

## UNITED STATES PATENT OFFICE.

BENJAMIN F. WALLACE, OF BROOKLYN, NEW YORK.

## COMPOUND FOR USE IN CASTING METALS.

No Drawing.

Application filed July 15, 1925. Serial No. 43,842.

This invention relates to the production of a so-called parting compound for employment in the casting of metals in order to effect a clean separation of the pattern from the sand surface in the mold, and has for its particular objects the production of a compound which is economical to manufacture and use, highly efficient, as well as possessing other advantages as hereinafter set forth.

For many years it has been customary in the foundry industry to employ dry parting powders approximating 200 mesh in fineness, which powders were dusted upon the pattern and surrounding sand surfaces between the cope and the drag. These parting powders commonly consisted of a silicious base, such as Tripoli rock, which is well known as essentially a natural decomposed silica, with which were incorporated varying percentages of vegetable oils, tallow, stearic acid and the like, by subjecting the mixture thereof for a relatively short period of time to a sufficient heat to cause the oil or fatty vehicle to become distributed over the surface of the particles and to thoroughly penetrate the same, whereby the resultant material becomes waterproof and will float for short periods of time on the water. The common test to determine when the heating operation is complete is to take test portions of the material and sprinkle the same on the surface of the water and if the same do not immediately sink upon the agitation of the water but it is only with difficulty that the surface tension of the particles is upset or affected with the resultant sinking of the particles, then it is recognized that the heating operation has been completed. Furthermore, the more impervious the mixture is to moisture and the more resistant such mixture is to having its surface tension affected when the same is floating on water and the surface agitated, the better the material is regarded for the purpose of effecting a perfect separation between the pattern and the sand in the operation of foundry molding.

The aforesaid Tripoli rock has been considered as an ideal base because of the fact that it is highly absorbent to fats and oils and thus rapidly becomes converted into a product possessing the necessary surface tension and water-repellent properties. These prior partings, whether having a Tripoli base or other similar base, were relatively very heavy as compared with my hereinafter de-

scribed product. For example, a barrel the size of the ordinary sugar barrel when packed therewith in the usual manner would weigh approximately 450 to 500 pounds; and the same barrel when mechanically packed, or as commonly expressed in the trade "when driven full", would weigh considerably more than this.

As a preferred example of my invention and the method of making the same, the following is set forth:

Precipitated calcium carbonate, which is a base that is ideally adapted for the production of parting because of its extreme fineness, its high grease and oil absorptive properties, and its extreme lightness, as well as because of the fact that the same constitutes a waste product in many industries, is first introduced while in a dry condition into a batch mixer, which latter is preferably provided with a suitable mechanical agitator or stirrer such as a shaft equipped with paddles or helical blades, or any other device designed to prevent the "balling up" of the mass during the mixing operation. This mixer is preferably heated either by the waste gases from a furnace or by the direct heat from a suitable furnace which may be located beneath the same. When the mixer containing the desired quantity of dry precipitated calcium carbonate, say one ton gross for example, has been thoroughly heated about 100 pounds of a suitable grease or oil mixture, such as for example melted tallow, stearic acid, melted degras grease or other melted fatty acid suitable for the purpose, is sprayed over the hot mass while the agitating devices are maintaining the same in a thoroughly agitated condition and the temperature of the batch is raised during such agitation to about 200 to 220 degrees C. A somewhat better distribution of the aforesaid grease, oil or fatty acids employed with the dry calcium carbonate may be obtained if a light solvent, such as kerosene for example, is employed to first dissolve the grease before spraying the same, in lieu of melting the same; then this thin mixture is sprayed on to the heated dry carbonate. The heating is continued until substantially all of the moisture has been vaporized and until the test sample when retested on the surface of the water will remain floating thereon despite continued and repeated jarring of the container, such as for example a test tube, in which the test is

made in an effort to dislodge the floating material on the surface in order to cause the same to sink.

In lieu of employing precipitated calcium carbonate in a substantially dry condition, I may also utilize the wet cake of precipitated calcium carbonate obtained from the filter press in various operations wherein the same is produced in a precipitated form, such for example as in the production of magnesia from Dolomite rock. Such filter press cake, which ordinarily will contain around 70% of water, is first introduced in the centrifuge wherein a substantial percentage of the water is removed and a product containing about fifty per cent of precipitated calcium carbonate and fifty per cent of water is obtained. This latter mass is then placed in the mixer aforesaid, and the grease, oil or fatty acid employed is directly introduced into the mixture without first heating the same or dissolving the same in a volatile solvent, and after such introduction the heat is applied to the mixture. The water is of course first vaporized from the mixture and the grease or oil vehicle is thoroughly distributed throughout the mass during such vaporization period and as soon as the water has been substantially driven off the thorough and intimate penetration of the grease or oil vehicle throughout the mass is effected in the same manner as when a dry precipitated calcium carbonate base is employed as above described. While this "wet process" requires a longer time for the production of a batch of the finished parting than does the above described dry process, nevertheless where the precipitated calcium carbonate is available in the form of a wet cake it eliminates the necessity and the expense of drying the same before its introduction into the mixture besides making it possible to maintain a more thorough distribution of the grease or oil vehicle throughout the batch, as not only is the heating and mixing operation of greater duration but also the wet, putty-like mass of this extremely light material tends to offer more resistance to the agitating devices, with the consequence that such vehicle becomes wrapped up more thoroughly and incorporated more effectively with the calcium carbonate base.

In order to further improve the product obtained as aforesaid and particularly to reduce to a minimum the tendency of the same to dust, which not only avoids waste but renders the air in the immediate vicinity of the molder better for inhalation into the lungs of the latter; and also in order to enhance the parting function of the material, especially in those cases where the molding sand is hot and steaming, I incorporate with the product produced by either of the methods above described a proportion of 1 to 5 per cent of kerosene oil prior to the removal of the same from the mixer but after the batch in such mixer

has been cooled to a point which is but slightly above the vaporizing point of the oil. Preferably such kerosene oil is sprayed into such batch, and the agitation is continued in the mixer until the kerosene oil has been thoroughly distributed throughout the mass. If desired, in lieu of such kerosene oil I may substitute for part or all of the kerosene oil other mineral or organic liquid solvents as gasoline or benzol (coal tar benzine), and may incorporate with such solvents varying percentages, preferably about 25%, of heavier hydrocarbons as petroleum residues, gas oil, waste, crank case oil from automobiles, or like compounds capable of imparting slipperiness properties to the parting.

Not only does the aforesaid treatment with kerosene or a mixture of kerosene and heavier hydrocarbon sufficiently reduce the dusting tendency of the finished product, but it also greatly facilitates the clean separation or parting of the pattern from the sand surface of the mold by virtue of the fact that it renders the finished product unctuous,—that is, it imparts thereto a greasy or soapy feel or "slip" and thus prevents the sticking of such product to the pattern as well as the consequent sticking of the sand to the latter. Owing to the natural dry, powdery consistency of calcium carbonate and its entire absence of unctuous property, as well as because of its high absorptive properties, this subsequent treatment to render the same unctuous is decidedly advantageous, as calcium carbonate is because of its high absorptive properties and lightness an ideal base for parting.

Because of the high absorptiveness of the carbonate base it is possible to render the same far more impervious and repellent to moisture than bases heretofore commonly employed, as Tripoli, burnt clay, fossil meal and the like, and as a consequence my improved product made as above described, particularly when employing either raw wool grease (degras) or refined wool grease (lanolin) as the waterproofing ingredient in the first step of the treatment, will remain floating on water for weeks and even months without settling, whereas parting products made from the other bases aforesaid sink usually within thirty-six to forty-eight hours when distributed on the surface of water. Furthermore, owing to its extreme fineness, which degree of fineness can only be approximated when employing silicious materials at a prohibitive expense for grinding the same, my improved product has a much greater covering or hiding power (i. e., pigment value) when dusted over the pattern and on the sand surface of a mold between the cope and the drag, with the consequence that notwithstanding its extremely light weight virtually the same volume or even less of my improved product will suffice for dusting the pattern and the sand surface as is now required with

a much heavier silicious base parting, with the consequence that my improved product is two to three times as efficient as other parting products now on the market.

5 Although I much prefer calcium carbonate as a base, my experiments have also led to the discovery that thoroughly calcined gypsum or precipitated calcium sulphate in such condition that it has lost its tendency to set 10 when mixed with water will also, when substituted for the aforesaid calcium carbonate and used in substantially the same proportions as such calcium carbonate in the above described methods of making parting, produce a very satisfactory parting and accordingly non-setting calcium sulphate is also included within the scope of certain of the appended claims as a base material of the parting covered thereby. Preferably in order to obtain a non-setting gypsum it is necessary to heat the same to approximately 500° C., for as is well known the partial de-hydration of gypsum results in the production of 20 plaster of Paris which latter product is unsuitable for the production of parting owing to its well-known setting properties when mixed with water.

While I have described the employment of 100 pounds of degras grease, either dissolved 30 in a suitable solvent or employed as such or in a melted condition, to one ton of calcium carbonate on a dry basis, or in other words, 5 per cent by weight of the base, it is obvious 35 that other percentages varying from two per cent to not over ten per cent may be employed without entirely losing the benefits of my invention, as the chief consideration in so far as the amount of waterproofing substance is concerned is to have a sufficient 40 quantity thereof to impart the necessary waterproofing properties while avoiding such an excess as would render the resultant parting objectionably sticky, to the extent that the same would tend to adhere to the pattern 45 as well as tend to cause "balling" of the product.

Likewise the proportions of kerosene oil employed in the final stage of the process might vary within wide limits, and if desired the same may be entirely substituted 50 by light lubricating oil or other oily compound adapted to impart the necessary unctuous properties to the finished product, but the percentage of such kerosene oil or oily material substituted therefor shall not be less 55 than one-half per cent, preferably not more than seven per cent, if the benefits thereof are to be properly secured. However, within 60 in the scope of certain of the appended claims is included a parting product which has not been subjected to the second stage of treatment with gasoline or like compound 65 capable of imparting unctuous properties to the compound, as for some purposes a product made in accordance with the first stage of the

herein described treatment has been found to be quite satisfactory.

My improved parting compound, whether made from precipitated calcium carbonate as a base or from thoroughly calcined non-setting gypsum ( $\text{CaSO}_4$ ), is remarkably light. The standard sugar barrel, the contents of which approximate six cubic feet, when filled with the same and loosely packed (i. e., not packed with a mechanical packer) 75 weighing somewhat less than 150 pounds, and when mechanically packed with a mechanical packer of the type provided with helical flights, weighing somewhat less than 200 pounds.

80 While I prefer to employ kerosene having a flashing point not under 150° C. for the second stage of the treatment either alone or in admixture with other oil vehicles, as well as employing the same in the first stage of the process in those cases where a volatile solvent is employed to dissolve the greasy material, nevertheless other solvents such as solvent naphtha, gasolene and the like may, if proper 85 precautions against fire are taken, be employed in lieu thereof, for the purpose of dissolving or thinning the grease or oil material employed in the first or second stages of the process.

Having thus described my invention, I 95 claim:

1. A parting composition for molds of foundries, comprising a finely divided precipitated alkaline-earth metal carbonate constituting its major ingredients, the same being 100 impregnated with a very small percentage of an organic waterproofing substance, said composition being extremely light and capable of floating on water without settling for long periods and in excess of fourteen days.

105 2. A parting composition for molds of foundries, comprising a finely precipitated calcium carbonate constituting its major ingredient, the same being impregnated with a very small percentage of an organic waterproofing substance, said composition being 110 extremely light and capable of floating on water without settling for long periods and in excess of fourteen days.

115 3. A molding composition for foundries, comprising a finely divided precipitated alkaline-earth metal carbonate constituting its major ingredient, the same being impregnated with a very small percentage of an organic waterproofing substance, said composition being 120 extremely light and capable of floating on water without settling for long periods and in excess of fourteen days, the particles having a superficial coating of such waterproofing substances to an extent sufficient to impart 125 thereto a decidedly greasy slip or feel and being substantially non-dusting.

130 4. A parting composition for molds of foundries, comprising a finely precipitated calcium carbonate constituting its major in-

- gradient, the same being impregnated with a very small percentage of wool grease, said composition being extremely light and capable of floating on water without settling for long periods and in excess of fourteen days.
5. A parting composition for molds of foundries, comprising a finely precipitated calcium carbonate constituting its major ingredient, the same being impregnated with about 5% of wool grease, said composition being extremely light and capable of floating on water without settling for long periods and in excess of fourteen days.
6. A parting composition for molds of foundries, comprising a finely precipitated calcium compound constituting its major ingredient, the same being impregnated with a very small percentage, and not exceeding ten percent, of an organic waterproofing substance, said composition being extremely light and capable of floating on water without settling for long periods and in excess of fourteen days.
7. The method of making a parting composition for molds of foundries which consists in impregnating an aqueous mass of a precipitated alkaline-earth metal carbonate base with a small percentage, and not exceeding ten percent, of an organic waterproofing substance and then subjecting the mass while agitating the same to heat sufficient to evaporate substantially all of the moisture and then continuing the heating operation during continued agitation thereof to a higher temperature to effect the thorough and homogeneous penetration of the waterproofing substance into the base.
8. The method of making a parting composition for molds of foundries which consists in impregnating an aqueous mass of a precipitated alkaline-earth metal carbonate base with a small percentage, and not exceeding ten percent, of an organic waterproofing substance and then subjecting the mass while agitating the same to heat sufficient to evaporate substantially all of the moisture and then continuing the heating operation during continued agitation thereof to a high temperature, and sufficient to effect the thorough and homogeneous penetration of the waterproofing substance into the base.
9. The method of making a parting composition for molds of foundries which consists in impregnating an aqueous mass of a precipitated alkaline-earth metal carbonate base with a small percentage, and not exceeding ten per cent, of an organic waterproofing substance and then subjecting the mass while agitating the same to heat sufficient to evaporate substantially all of the moisture and then continuing the heating operation during continued agitation thereof to a high temperature, of at least 200° C.
10. The method of making a parting composition for molds of foundries which con-
- sists in impregnating an aqueous mass of a precipitated alkaline-earth metal carbonate base with a small percentage, and not exceeding seven per cent, of an organic waterproofing substance and then subjecting the mass while agitating the same to heat sufficient to evaporate substantially all of the moisture, then continuing the heating operation during continued agitation thereof to a higher temperature to effect the thorough and homogeneous penetration of the waterproofing substance into the base, and then allowing the mass to cool and distributing throughout the mass a small percentage of volatile hydrocarbon solvent while the temperature of said mass is still substantially above the vaporizing point of such solvent.
11. The method of making a parting composition for molds of foundries which consists in impregnating an aqueous mass of a precipitated alkaline-earth metal carbonate base with a small percentage, and not exceeding ten per cent, of an organic waterproofing substance and then subjecting the mass while agitating the same to heat sufficient to evaporate substantially all of the moisture, then continuing the heating operation during continued agitation thereof to a higher temperature to effect the thorough and homogeneous penetration of the waterproofing substance into the base, and then spraying the mass after the partial cooling of same with small percentage of a mixture of kerosene and heavier hydrocarbons.
12. The method of making a parting composition for molds of foundries which consists in impregnating an aqueous mass of a precipitated alkaline-earth metal carbonate base with a small percentage, and not exceeding ten per cent, of an organic waterproofing substance and then subjecting the mass while agitating the same to heat sufficient to evaporate substantially all of the moisture, then continuing the heating operation during continued agitation thereof to a higher temperature to effect the thorough and homogeneous penetration of the waterproofing substance into the base, and then distributing throughout the mass while still hot small percentage of a hydrocarbon liquid adapted to substantially eliminate objectionable dusting of the finished product when in use and to impart a greasy "slip" to the particles thereof wherein in use the sticking of the same to the pattern, with the consequent sticking of the same to the latter, is prevented.
13. In the manufacture of a molding composition for foundries, the step which consists in superficially coating a grease impregnated highly absorbent, fluffy, water-insoluble salt of calcium with a small percentage, and not exceeding seven per cent, of an oily substance to allay the dusting thereof and to render the same unctuous.
14. In the manufacture of a molding com-

position for foundries, the step which consists in spraying a base comprising calcium carbonate, homogeneously impregnated with degras grease, with a small percentage, and 10  
5 not exceeding seven per cent, of kerosene.

15. In the manufacture of a molding composition for foundries, the step which consists in spraying a base comprising calcium

carbonate, homogeneously impregnated with degras grease, with a small percentage, and 10  
not exceeding seven per cent of a mineral oil.

Signed at New York, in the county of New York and State of New York, this 14th day of July, 1925.

BENJAMIN F. WALLACE.